

Patented Feb. 9, 1926.

## UNITED STATES PATENT OFFICE.

JOHN C. BLACK, OF DESTREHAN, LOUISIANA, AND JAMES W. WEIR, OF FILLMORE, CALIFORNIA.

## PROCESS FOR MANUFACTURING LUBRICATING OILS.

No Drawing.

Application filed October 19, 1922. Serial No. 595,660.

To all whom it may concern:

Be it known that we, JOHN C. BLACK, a citizen of the United States, residing at Destrehan, in the parish of Saint Charles, State of Louisiana, and JAMES W. WEIR, a citizen of the United States, residing at Fillmore, in the county of Ventura, State of California, have invented certain new and useful Improvements in a Process for 10 Manufacturing Lubricating Oils, of which the following is a specification.

This invention relates to the art of refining petroleum or petroleum distillates, or other hydrocarbons, and more specifically to 15 those petroleum products known as lubricating oils.

The object of this invention is to facilitate treatment of the oil and to increase the yield of finished products, and to improve 20 the quality of such finished products in its color and other physical characteristics, and to eliminate certain steps in the treatment of the oils as heretofore practiced in the manufacture of lubricating oils.

25 Heretofore in the refining of lubricating oils, it was the custom to treat the oils with sulphuric acid, withdraw the acid reaction products as completely as practical, then neutralize the remaining acid reaction products with caustic soda solution or other 30 neutralizing agent, and then washing out the remaining neutralizing agent or its products with water, after which it may be brightened by blowing it with air. After 35 this treatment the color is not usually up to the standard desired and will be further subjected to a decolorizing treatment either by percolation or contact with fuller's earth or other decolorizing substance to bring the 40 finished product to the color desired.

By our new and improved method we have discovered a procedure whereby several of the foregoing individual steps may be eliminated, and more particularly the one 45 of neutralization with caustic soda and the following step of washing with water, and also the further step of decolorization as an independent operation as heretofore.

Our procedure in treating or refining 50 lubricating oil is as follows:

The oil is first given an acid treatment, preferably with sulphuric acid, in the manner usually employed; the resulting sludge acid is then removed; the oil is then

in condition for final treatment which consists in admixing a finely divided clay, fuller's earth, montmorillonite, infusorial earth, silica gel, or similar substance, which may be either in a raw condition or treated by any of the well known treating processes 55 to increase the adsorbing surface of the substance; sufficient of the reagent as enumerated above is added to the oil to accomplish in one operation the neutralization and decolorization of the oil with the consequent 60 elimination of the neutralization step with caustic soda, the washing with water, the brightening step, and also the decolorization by percolation or contact as a separate step. This procedure eliminates the expensive 65 caustic soda treatment and also the loss of yield of oil by the soda wash and subsequent water wash. It also eliminates the production of oil soluble soda soaps detrimental 70 in the best quality lubricating oils. 75

We have further discovered that to completely neutralize the oil by this method that it is necessary to heat the oil with the admixed neutralizing and decolorizing agent to drive off the final acid reaction products 80 that are in the form of sulphur dioxide. To accomplish this, we heat the mixture, while under treatment, to at least 180° F., but preferably above the boiling point of water. The heating, we have discovered, has a two-fold function, first to drive off the SO<sub>2</sub> 85 products of reaction, and secondly, to increase the decolorization action of the neutralizing and decolorizing reagent. Furthermore, we have discovered that the SO<sub>2</sub> gas 90 is beneficial in the decolorization reaction in that it forms a non-oxidizing atmosphere in contact with the oil and prevents darkening 95 of the oil by oxidation.

After the neutralization and decolorization step is complete, the oil is separated from the neutralizing and decolorizing reagent by any of the well known methods of separation of a liquid and a finely divided mineral substance; the separation may be 100 made while the oil is heated, or it may be made after cooling or during cooling. The cooling of the oil should preferably be performed in a closed cooling apparatus from which air is excluded to prevent oxidation 105 and darkening of the oil.

If it is found that the finished oil is cloudy due to moisture, it may be removed by only

partially cooling the oil to 180° F. or lower and blowing air or an inert gas through the oil. This will brighten the oil due to the air or gas being undersaturated at the temperature employed and will therefore take up moisture approaching its saturation point.

- In practice, after neutralizing the oil as described in the Weir Patent No. 1,564,501, 10 if a lighter colored oil were required it would be necessary to make a further decolorizing step, using a decolorizing clay, in order to produce an oil of the same color as that which could be made by the process of 15 Black and Weir under their joint specification. Where under the Weir process as patented he uses 5,000 gallons of oil to one ton of clay and produces a neutralized oil of 3½ color (N. P. A.), which is the color obtained 20 by the acid alone, under the process of the joint application of Black and Weir 2,500 gallons of oil to one ton of clay would be used and an oil of about 3 color (N. P. A.) would be produced if a decolorizing clay 25 were used. This 3 color oil would be an oil materially lighter in color and have a higher market value.

To summarize and make clear our preferred method of operation, we will outline 30 the procedure as follows:

The oil is first treated with sulphuric acid; the sludge acid is allowed to settle, and is withdrawn or separated from the oil; the oil is then admixed with the neutralizing 35 and decolorizing reagent and the mixture heated to 180° F. or higher until the oil is neutral and the proper discolorization obtained; the mixture is then discharged through a filter and cooled and finally discharged to storage. The filtering and cooling 40 steps may be reversed, but we prefer to filter then cool, as we find this facilitates the operation. If the oil is cloudy, it may be brightened as previously described.

We claim:

1. A method of refining hydrocarbons consisting in treating the hydrocarbons with sulphuric acid; withdrawing the precipitated acid reaction products, adding to the treated hydrocarbons a neutralizing and decolorizing reagent in sufficient quantities to decolorize the hydrocarbons and heating the mixture, then separating the hydrocarbons and admixed reagent.
2. A method of refining hydrocarbons consisting in treating the hydrocarbons with sulphuric acid, withdrawing the precipitated acid reaction products, adding to the treated hydrocarbons a neutralizing and decolorizing reagent in sufficient quantities to decolorize the hydrocarbons and heating the mixture to above 180° F., then separating the hydrocarbons and admixed reagent.
3. A method of refining hydrocarbons 65 consisting in treating the hydrocarbons

with sulphuric acid, withdrawing the precipitated acid reaction products, adding to the treated hydrocarbons a neutralizing and decolorizing reagent in sufficient quantities to decolorize the hydrocarbons and heating 70 the mixture, and while heated separating the hydrocarbons and admixed reagent, then cooling the hydrocarbons.

4. A method of refining hydrocarbons consisting in treating the hydrocarbons 75 with sulphuric acid, withdrawing the precipitated acid reaction products, adding to the treated hydrocarbons a neutralizing and decolorizing reagent in sufficient quantities to decolorize the hydrocarbons and heating 80 the mixture to above 180° F., separating the hydrocarbons and admixed reagent, then cooling the hydrocarbons to materially less than 180° F.

5. A method of refining hydrocarbons 85 consisting in treating hydrocarbons with sulphuric acid, withdrawing the precipitated acid reaction products, adding to the treating hydrocarbons neutralizing and decolorizing reagents in sufficient quantities 90 to decolorize the hydrocarbons and heating the mixture, then filtering the hydrocarbons to separate the admixed reagent.

6. A method of refining hydrocarbons 95 consisting in treating the hydrocarbons with sulphuric acid, withdrawing the precipitated acid reaction products, adding to the treated hydrocarbons, neutralizing and decolorizing reagents in sufficient quantities 100 to decolorize the hydrocarbons and simultaneously heating the mixture to approximately above 180° F., then cooling the mixture below 180° F. and separating the hydrocarbons and admixed reagent then cooling 105 the hydrocarbons.

7. A method of refining hydrocarbons consisting in treating the hydrocarbons with sulphuric acid, withdrawing the precipitated acid reaction products, adding to the treated hydrocarbons; neutralizing and decolorizing reagents in sufficient quantities to decolorize the hydrocarbons and heating the mixture, separating the hydrocarbons and admixed reagent, then brightening by 110 blowing a gas through them.

8. A method of refining hydrocarbons consisting in treating the hydrocarbons with a sulphuric acid, withdrawing the precipitated acid reaction products, adding to the treated hydrocarbons neutralizing and decolorizing reagents in sufficient quantities to decolorize the hydrocarbons and heating the mixture to above 180°, separating the hydrocarbons and admixed reagent, cooling the hydrocarbons to materially less than 180° F., then brightening them.

9. A process of neutralizing and decolorizing hydrocarbon containing acid reaction products consisting in first withdrawing the acid reaction products then adding neutral-

izing and decolorizing reagents, in sufficient quantities to neutralize and decolorize the hydrocarbon, then heating the mixture of hydrocarbon, acid reaction products and neutralizing and decolorizing reagents to an active reaction temperature, then separating the admixed reagents together with the reaction products from the decolorized hydrocarbon.

10 10. The method of refining hydrocarbons containing acid reaction products which comprises first removing the said re-

action products, then adding a comminuted decolorizing agent to the hydrocarbons in sufficient quantities to both neutralize and decolorize the hydrocarbons, heating the mixture to above 180° Fahrenheit, and separating the adsorbent material with the materials adsorbed thereon from the oil stock.

15 In testimony whereof we have signed our names to this specification.

JOHN C. BLACK.  
JAMES W. WEIR.